

## UNITED STATES PATENT OFFICE

LUDWIG LOCK, OF DORMAGEN-ON-THE-RHINE, GERMANY, ASSIGNOR TO I. G. FARBEN-INDUSTRIE AKTIENGESELLSCHAFT, OF FRANKFORT-ON-THE-MAIN, GERMANY, A CORPORATION OF GERMANY

## PROCESS OF MAKING CELLULOSE NITRO ACETATE

No Drawing. Application filed September 12, 1929, Serial No. 392,257, and in Germany September 19, 1929.

The present invention relates to a process of preparing cellulose nitro acetates.

The manufacture of cellulose nitro acetates has hitherto been carried out in two separate processes. Thus, for example, according to the process of the German Patent No. 295,889, the bleached cellulose serving as the starting material is preliminarily nitrated by a mild treatment with a weakly acting 10 nitrating acid mixture, for example, to a nitrogen content of 2%, freed from adhering acid, washed and dried, after which acetylation is effected in the second stage of the process by one of the known technical 15 methods.

The present invention describes a new process of producing cellulose nitro acetates in one and the same process in a technically easy and simple manner. The process consists in acetylating the cellulose at temperatures between about 50 and 100° C. by means of acetic acid and acetic anhydride in the presence of a calculated amount of a salt of nitric acid with a weak inorganic or organic 20 base, such as for example ammonium nitrate, zinc nitrate, aniline nitrate and urea nitrate, with the addition of a small amount, say about 0.2-1% calculated on the amount of the cellulose to be acylated, of a free 25 mineral acid, especially sulfuric acid. The quantity of the salt of the nitric acid to be added to the reaction mixture depends on the desired nitrogen content of the cellulose nitro acetate to be prepared. Thus, there 30 are obtainable cellulose nitro acetates with a nitrogen content of about 0.1 to 1.8%.

In addition to the extraordinarily valuable effect of having combined two expensive 35 separate processes into a single reaction, which is readily and securely carried out the new and technically equally important feature must be considered of being able to predetermine in this manner the nitrogen content of the ultimate cellulose nitroacetate.

The nitro acetates obtained in this manner are extraordinarily clear and viscous and form a valuable material for the film industry, which is distinguished among others 40 from the products obtained from non-ni-

trated cellulose acetate by a considerably reduced water stretchability.

The invention is illustrated by the following examples, without being limited thereto:

*Example 1.*—One part by weight of cellulose is heated at 70° C. with 5 parts by weight of acetic anhydride, 3 parts by weight of glacial acetic acid and 0.05 parts by weight of ammonium nitrate with the addition of 0.003 parts by weight of sulfuric acid until a test portion is found to be soluble in chloroform. The triacetate contains 0.6% of nitrogen (calculated on the cellulose). The resulting nitro acetate is then hydrolyzed according to one of the known processes.

*Example 2.*—One part by weight of cellulose is heated at 100° C. with 4 parts by weight of acetic anhydride, 2 parts by weight of glacial acetic acid and 0.5 parts by weight of ammonium nitrate with the addition of 0.004 parts by weight of sulfuric acid until a test portion is found to be soluble in chloroform. The triacetate contains 1.5% of nitrogen calculated on the cellulose. It is then hydrolyzed according to one of the known processes.

*Example 3.*—One part by weight of cellulose is heated at 80° C. with 3 parts by weight of acetic anhydride, 3 parts by weight of glacial acetic acid and 0.1 part by weight of urea nitrate with the addition of 0.005 parts by weight of sulfuric acid until a test portion is found to be soluble in chloroform. The triacetate contains 0.8% of nitrogen, (calculated on the cellulose); it is then hydrolyzed according to one of the known processes.

I claim:

1. The process which comprises acetylating cellulose between about 50 and 100° C. by means of acetic acid and acetic anhydride in the presence of a small amount of mineral acid and of a salt of nitric acid with a weak base.

2. The process which comprises acetylating cellulose between about 50 and 100° C. by means of acetic acid and acetic anhydride in the presence of a small amount of sulfuric acid and of a salt of nitric acid with a weak base.

3. The process which comprises acetylating cellulose between about 50 and 100° C. by means of acetic acid and acetic anhydride in the presence of 0.2-1% (calculated on the amount of the cellulose) of sulfuric acid and of a salt of nitric acid with a weak base.
4. The process which comprises acetylating cellulose between about 50 and 100° C. by means of acetic acid and acetic anhydride in the presence of 0.2-1% (calculated on the amount of the cellulose) of sulfuric acid and of urea nitrate.

In testimony whereof, I affix my signature.  
LUDWIG LOCK.